

## UNITED STATES PATENT OFFICE

2,289,365

## IRON-PHOSPHORUS-SILICON ALLOY

Henry S. Jerabek, Minneapolis, Minn.

No Drawing. Application August 29, 1941,  
Serial No. 408,859

12 Claims. (Cl. 75—123)

(Granted under the act of March 3, 1883, as  
amended April 30, 1928; 370 O. G. 757)

The invention herein described may be manufactured and used by or for the Government for governmental purposes without the payment to me of any royalty thereon.

This invention relates to ferrous alloys and, more particularly, to iron-phosphorus-silicon alloys which have good properties in regard to casting and corrosion resistance of articles produced therefrom.

During the reduction of phosphate charging stocks to produce elemental phosphorus a certain proportion of an iron-phosphorus alloy containing varying proportions of minor constituents is produced. Even the proportions of the principal constituents vary considerably, depending upon the conditions of operation of the phosphate reduction furnace in which they are produced. These iron-phosphorus alloys are useful to a limited extent in the production of steels, but the further utilization of such alloys in substantial proportions to produce useful articles of manufacture has not hitherto been particularly promising.

The alloys of the present invention are composed of the following essential constituents in approximately the proportions stated: 2 to 13% phosphorus, 6 to 22% silicon, the total of the phosphorus and silicon being not more than approximately 26%, with the balance substantially all iron. Alloys conforming to the above composition may contain up to 35% of a metal selected from the group consisting of aluminum, chromium, copper, manganese, molybdenum, nickel, titanium, and vanadium substituted for part of such iron.

A preferred narrower range of the essential constituents is as follows: 5 to 10% phosphorus, 10 to 15% silicon, with the balance substantially all iron, or up to 25% of a metal selected from the foregoing group substituted for a part of the iron.

The alloys of the present invention are suitable for casting to form articles of manufacture which are particularly corrosion resistant and, therefore, suitable for producing articles such as acid pumps, acid conduits, and the like. The alloys so produced have been found particularly resistant to attack in contact with 80% orthophosphoric acid at 240° F., 90% orthophosphoric acid

at 280° F., boiling 20% hydrochloric acid, and boiling 30% sulfuric acid.

Ferrophosphorus produced under a wide range, plant scale, phosphate reduction furnace operation has been found to have the following approximate compositions:

| P        | Si       | Mn       |
|----------|----------|----------|
| Per cent | Per cent | Per cent |
| 26.2     | Trace    |          |
| 25.0     | 0.4      |          |
| 25.2     | 1.0      | 3.2      |
| 19.7     | 8.2      | 3.4      |
| 16.6     | 12.1     |          |
| 13.5     | 15.8     |          |
| 13.4     | 17.2     |          |
| 12.2     | 19.4     |          |

The impurities which are present in all electric furnace ferrophosphorus are shown by the following typical analyses:

| P    | Si   | Mn  | Ti  | Al  | C   | S   |
|------|------|-----|-----|-----|-----|-----|
| 13.7 | 17.5 | 3.5 | 1.0 | 0.1 | Tr. | Tr. |
| 17.4 | 12.7 | 3.5 | 1.3 | 0.2 | Tr. | Tr. |
| 25.1 | 0.9  | 3.5 | 1.1 | 0.2 | Tr. | Tr. |

Such commercial ferrophosphorus has been used to produce the alloys of the present invention in conjunction with other metals or alloys as follows:

*Armco ingot iron.*—Typical analysis—99.78 per cent Fe, 0.013 per cent C, 0.02 per cent Mn, 0.002 per cent P, 0.001 per cent Si, 0.04 per cent Cu, and 0.02 per cent Ni.

*Silicon.*—Analysis—99.79 per cent Si, 0.027 per cent Fe, 0.003 per cent Al, 0.014 per cent Ca, 0.004 per cent C, 0.10 per cent N<sub>2</sub>.

*Low-carbon ferrochrome.*—71.5 per cent Cr, 0.16 per cent C (60 mesh).

*Nickel shot (98-99 per cent Ni).*—Analysis—0.4-0.7 per cent Fe, 0.1-0.3 per cent Cu, 0.15-0.6 per cent C, 0.15-0.3 per cent Si.

*Copper.*—High conductivity grade 99.8+ per cent Cu—typical analysis.

*Molybdenum.*—Powdered.

*Ferrovanadium (51 per cent V).*—Typical analysis—6 per cent Mn, 10 per cent Si, 1.6 per cent C, 1 per cent S.

Charges of predetermined composition were melted in a zircon lined alundum or graphite crucible and poured into open top cast iron molds. Castings were removed quickly from the mold while red hot and placed in a muffle furnace for cooling slowly to room temperature. It appears that such cooling is necessary to properly anneal the castings and thereby avoid the production of undue internal stress.

Compositions having the essential components in approximately the following proportions have been found by test to have especially desirable properties in regard to casting and corrosion resistance of cast articles made therefrom:

| Alloy No. | Composition |          |         |
|-----------|-------------|----------|---------|
| 22        | 7.5% P      | 12.5% Si | 15% Cu  |
| 34        | 7.5% P      | 12.5% Si | 25% Cr  |
| 35        | 7.5% P      | 12.5% Si | 1% V    |
| 36        | 7.5% P      | 12.5% Si | 3% Mo   |
| 37        | 7.5% P      | 12.5% Si | 15% Ni  |
| 41        | 7.5% P      | 12.5% Si | -----   |
| 42-42A    | 7.5% P      | 12.5% Si | -----   |
| 45        | 8% P        | 9% Si    | -----   |
| 47-47A    | 7.5% P      | 12.5% Si | Tr. Cr  |
|           | 7.3% P      | 14.0% Si | 2.2% Mo |

Impact tests on specimens of alloys Nos. 42, 42A, 45, 47 and the last alloy in the immediately preceding table in a Charpy impact machine showed foot pounds absorbed 5, 2, 1, 2.4 and 3.6, respectively, using 10 x 10 x 510 mm. specimens, with a notch 1 mm. deep and 1.5 mm. radius. Hardness tests on alloys Nos. 42, 42A, 45, 47 and 47A by a Shore scleriscope gave an average Shore hardness number of 91, 96, 72, 96 and 94, respectively. These latter results may be compared with those values for properly hardened tool steel, 91 Shore, and Stellite, 85 Shore. These specimens were too brittle for Rockwell tests.

I claim:

1. An alloy comprising the following elements in approximately the proportions given
  - (a) 2 to 13% phosphorus,
  - (b) 6 to 22% silicon, the total of the phosphorus and silicon being not more than approximately 26%,
  - (c) the balance substantially all iron.
2. A corrosion resistant article of manufacture formed of a metal alloy comprising the following elements in approximately the proportions given
  - (a) 2 to 13% phosphorus,
  - (b) 6 to 22% silicon, the total of the phosphorus and silicon being not more than approximately 26%,
  - (c) the balance substantially all iron.
3. An alloy comprising the following elements in approximately the proportions given
  - (a) 7.5% phosphorus,
  - (b) 12.5% silicon,
  - (c) the balance substantially all iron.
4. An alloy comprising the following elements in approximately the proportions given
  - (a) 7.5% phosphorus,
  - (b) 12.5% silicon,
  - (c) 3% molybdenum,
  - (d) the balance substantially all iron.

5. An alloy comprising the following elements in approximately the proportions given

- (a) 2 to 13% phosphorus,
- (b) 6 to 22% silicon, the total of the phosphorus and silicon being not more than approximately 26% and
- (c) up to 35% aluminum,
- (d) the balance substantially all iron.

6. An alloy comprising the following elements in approximately the proportions given

- (a) 2 to 13% phosphorus
- (b) 6 to 22% silicon, the total of the phosphorus and silicon being not more than approximately 26% and

15 (c) up to 35% chromium,

- (d) the balance substantially all iron.

7. An alloy comprising the following elements in approximately the proportions given

- (a) 2 to 13% phosphorus,
- (b) 6 to 22% silicon, the total of the phosphorus and silicon being not more than approximately 26% and
- (c) up to 35% copper,
- (d) the balance substantially all iron.

20 8. An alloy comprising the following elements in approximately the proportions given

- (a) 2 to 13% phosphorus,
- (b) 6 to 22% silicon, the total of the phosphorus and silicon being not more than approximately 26% and
- (c) up to 35% manganese,
- (d) the balance substantially all iron.

30 9. An alloy comprising the following elements in approximately the proportions given

- (a) 2 to 13% phosphorus,
- (b) 6 to 22% silicon, the total of the phosphorus and silicon being not more than approximately 26% and
- (c) up to 35% molybdenum,
- (d) the balance substantially all iron.

40 10. An alloy comprising the following elements in approximately the proportions given

- (a) 2 to 13% phosphorus,
- (b) 6 to 22% silicon, the total of the phosphorus and silicon being not more than approximately 26% and
- (c) up to 35% nickel,
- (d) the balance substantially all iron.

45 11. An alloy comprising the following elements in approximately the proportions given

- (a) 2 to 13% phosphorus,
- (b) 6 to 22% silicon, the total of the phosphorus and silicon being not more than approximately 26% and
- (c) up to 35% titanium,
- (d) the balance substantially all iron.

55 12. An alloy comprising the following elements in approximately the proportions given

- (a) 2 to 13% phosphorus,
- (b) 6 to 22% silicon, the total of the phosphorus and silicon being not more than approximately 26% and
- (c) up to 35% vanadium,
- (d) the balance substantially all iron.